

1

2,875,029

## STABILIZED LIQUID FUEL

Leo A. McReynolds, Bartlesville, Okla., assignor to Phillips Petroleum Company, a corporation of Delaware

No Drawing. Application May 21, 1953  
Serial No. 356,589

6 Claims. (Cl. 44—70)

This invention relates to the stabilization of liquid hydrocarbon fuels. In one of its more specific aspects, the invention relates to the prevention of gum formation in liquid fuels. In another of its more specific aspects, the invention relates to the prevention of gum formation in liquid fuels during periods of storage, especially under the influence of light and/or oxygen.

It is well known that when liquid fuels such as gasoline, diesel fuel, jet fuel, fuel oil and the like, are stored, especially under the influence of light and/or oxygen, chemical changes occur which affect the color and increase the gum formation. Gum formation in liquid fuels adversely affects the operation of equipment in which such fuels are used, such as internal combustion engines, domestic and industrial burner systems, etc., by clogging feed lines, screens, nozzles and the like. It is conventional practice to add gum inhibitors to hydrocarbon materials ranging from the gasoline boiling range through the furnace oils and diesel fuels range. The hydrocarbon fuels which contain large amounts of cracked distillates are particularly subject to the problem of gum formation.

Each of the following objects will be attained by at least one of the aspects of this invention.

An object of this invention is to provide a stabilized liquid fuel. Another object of the invention is to provide a liquid fuel stabilized by the addition of a minor portion of a product of the oxidation of selected high molecular weight hydrocarbons to such fuel. Another object of the invention is to provide a method for enhancing storage stability of liquid hydrocarbon fuels.

Other and further objects of this invention will be apparent to those skilled in the art upon study of the accompanying disclosure.

Broadly speaking, this invention comprises the stabilization of liquid hydrocarbon fuels by the addition thereto of between 0.0001 and 0.1 weight percent based on the liquid hydrocarbon, preferably between 0.001 and 0.01 weight percent of a product of the oxidation of a selected hydrocarbon fraction having at least 40 carbon atoms per molecule. The selected hydrocarbon material should have a refractive index of between 1.440 and 1.520. Hydrocarbon material which may be satisfactorily used in the preparation of this additive includes substantially saturated diene polymers, such as polybutadiene, and olefin polymers having from 2 to 12 carbon atoms per monomer molecule, such as polypentadiene, polypropylene, polyethylene, polyisobutylene, etc., preferably having a ratio of carbon atoms to olefin bonds of at least 40:1 and not less than 16:1, copolymers such as styrene-olefin copolymers, alkylated polystyrene, and a petroleum lubricating oil fraction which has substantially no asphalt within its natural state or when deasphalted and which has been solvent extracted to reduce the content of aromatic hydrocarbons therein and preferably dewaxed. Petroleum fractions which are suitable for oxidation to produce the stabilizing additive, i. e., a stabilizer for normally liquid hydrocarbon fuels ranging from the gasoline boiling range to about 720° F., preferably the furnace oils and fuel oils

2

boiling in the range of about 380° F. to 640° F., include Pennsylvania, Mid-Continent, California, East Texas, Gulf Coast, Venezuela, Borneo, and Arabic crudes. The source of the crude from which the petroleum fraction is derived does not significantly influence the preparation or properties of the stabilizing additive, provided the petroleum fraction has been prepared by subjecting the crude to certain necessary treatments to exclude undesired materials therefrom.

10 In the preparation of the preferred petroleum fraction from which the stabilizing additive is produced, a crude oil is topped, i. e., distilled to remove therefrom the more volatile, lower molecular weight hydrocarbons such as gasoline and light gas oil, and then vacuum reduced to remove heavy gas oil and light lubricating oil of the SAE 10 and 20 viscosity grade. The vacuum reduced crude is then propane fractionated to remove an overhead fraction of about 100 SUS at 210° F. viscosity. The residue from the second fractionation may be subjected to a propane fractionation to remove still another overhead fraction of about 575 SUS at 210° F. viscosity. Propane fractionation may be modified by the presence of butane, ethane, or methane to the extent desired.

Following the propane fractionation step the overhead oil fraction is solvent extracted with a selective solvent which will separate the paraffinic hydrocarbons from the more aromatic-type hydrocarbons. Suitable selective solvents for aromatic hydrocarbons include among others the various phenols, sulfur dioxide, furfural and  $\beta,\beta'$ -dichlorodiethyl ether. This solvent extraction step for the removal of the more highly aromatic compounds can be carried out in accordance with the well-known concurrent or countercurrent solvent extraction techniques as well as by the well-known dual solvent technique.

35 The resulting solvent extracted material, before or after the removal of the more aromatic hydrocarbons, is preferably dewaxed. Dewaxing may be carried out by any conventional method, e. g., by solvent dewaxing using propane or solvent mixture such as methyl ethyl ketone or methyl isobutyl ketone with benzene at a suitable temperature.

Each of the phenol extracted, dewaxed, propane-fractionated oils have been used in preparing the additive material of this invention with good results but the oil fraction from the second propane fractionation is preferred. It will be recognized by those skilled in the art that propane fractionated oils differing from those described may be used or a single broad viscosity cut can be used. The residual material from the final propane fractionation contains the rejected asphalt and more aromatic oils.

50 Although the preferred method for preparation of feed stock is as above described, other methods may be used to secure a similar type hydrocarbon fraction. Thus, a vacuum reduced crude which has essentially no asphalt, such as a Pennsylvania oil, may be used directly or after a light acid treatment. Another method, while not feasible commercially at the present time, is ultra-high vacuum (molecular) distillation to obtain the desired fraction described more exactly in subsequent paragraphs.

60 As pointed out above, a polydiene such as liquid polybutadiene which is prepared by sodium-catalyzed polymerization of butadiene and which material is subsequently hydrogenated so as to reduce the olefinic unsaturation thereof to a desired amount, is another suitable feed stock for use in the production of the additive material of this invention. When butadiene is polymerized, only one double bond remains therein for each butadiene group of the polymer. The feed material of this invention should be hydrogenated sufficiently so that the ratio of carbon atoms to double bonds is at least 16 to 1. Preparation of liquid polybutadiene may be obtained by means of the process set forth in U. S. application Serial No. 67,098, filed De-

ember 23, 1948, by W. W. Crouch, now Patent No. 2,631,175, issued March 10, 1953.

Another suitable feed stock is a liquid or semi-solid polybutadiene which is prepared by conventional emulsion polymerization and coagulation to form synthetic rubber and which material is subsequently hydrogenated so as to reduce the olefinic unsaturation thereof to the desired amount and finally thermally depolymerized sufficiently to increase the ease of oxidation and to increase the oil solubility.

Another suitable feed material is a high molecular weight polymer prepared by zirconium tetrachloride polymerization of propylene. Still another material which has proved to be useful as a feed material for the oxidation step in the preparation of the additive material of this invention is a "tacky polymer" prepared by the polymerization of propylene over chromia-silica-alumina catalyst as more fully disclosed in U. S. application Serial No. 333,576, filed January 27, 1953, by John P. Hogan and Robert L. Banks, now abandoned (see U. S. Patent 2,825,721, March 4, 1958). Another suitable feed material is a copolymer of styrene with olefins in which the olefin portion constitutes at least 50 percent of the total molecular weight of the molecule. With any of these feed materials, it is desired to reduce the amount of olefinic unsaturation to such an extent that the ratio of carbon atoms to olefinic bonds is preferably at least 40:1 and not less than 16:1. The hydrocarbon stocks which are useful in the practice of this invention include those materials which are identifiable as having the following properties set forth in Table 1.

TABLE 1

| Property                                         | Broad Range | Preferred Range |
|--------------------------------------------------|-------------|-----------------|
| Refractive Index $n_D^{20}$                      | 1.440-1.520 | 1.480-1.515     |
| Average Molecular Weight                         | above 550   | 600-10,000      |
| Minimum Molecular Weight                         | 450         |                 |
| Viscosity, SUS at 210° F.                        | above 50    | above 100       |
| Viscosity Index (when determinable) <sup>1</sup> | 50-125      | 80-120          |
| Carbon Atom Content per Molecule                 | above 40    | 50-720          |

<sup>1</sup> Viscosity index not determinable for non-Newtonian materials.

The lubricating oil and polymers having a similar viscosity which are suitable as feed stocks for the production of the oxidation product used as the stabilized additive of my invention, are set forth as follows in Table 2.

TABLE 2

| Property                         | Broad Range | Preferred Range |
|----------------------------------|-------------|-----------------|
| Refractive Index $n_D^{20}$      | 1.440-1.520 | 1.480-1.515     |
| Average Molecular Weight         | 550-1,300   | 600-900         |
| Minimum Molecular Weight         | 450         |                 |
| Viscosity, SUS at 210° F.        | 50-1,400    | 100-600         |
| Viscosity Index                  | 50-125      | 80-120          |
| Carbon Atom Content per Molecule | 40-80       | 50-70           |

It appears that during oxidation, scission takes place in the large hydrocarbon molecules. This is substantiated by passing nitrogen gas through the oil at 250° C. and collecting the volatile products which were negligible. Only a very small amount was collected when the temperature was raised to 300° C., thus demonstrating that the major cause of the formation of the volatile products is oxidation and not thermal decomposition nor stripping of light ends originally present in the oil. With oils of moderate molecular weight, scission cannot take place in any position but what one or all of the fragments is sufficiently small that distillation takes place, thus preventing accumulation of molecules appreciably smaller than those originally present. Hence, the viscosity is not decreased to any great extent. Concomitant with the oxidative scission reaction there is a polymerization or condensation reaction resulting in an increase in viscosity. The net change in viscosity is apparently due to the relative

magnitude of each reaction. In very high molecular weight hydrocarbons the oxidative scission more frequently results in fragments which have molecular weights too large to be removed by distillation and, hence, the molecular weight decreases causing a decrease in viscosity especially during the initial portions of the oxidation period. As the oxidation reaction proceeds, the reactions causing increased molecular weight may offset, more or less, those causing a decrease in molecular weight. As a result, the molecular weights of charge oils having molecular weights in the lower range tend to increase and those in the higher range tend to decrease during the initial oxidation period.

If desired, the petroleum oil fraction which has been highly refined as described above may be further subjected to additional refining treatments, for example, these petroleum fractions may be hydrogenated to convert any aromatic compounds therein to the corresponding naphthenic and saturated hydrocarbon, or if desired, these petroleum fractions may be subjected to contact with silica gel for the preferential adsorption and removal of the more aromatic hydrocarbons therefrom. Generally, the petroleum fraction which is oxidized for the production of the stabilizing additive of this invention should contain not more than 20 percent of the carbon atoms in aromatic rings as determined by ring analysis. It is preferred that the aromatic content of the petroleum fraction be reduced to an economically feasible extent by refining procedures since oxidation of aromatic type hydrocarbons tend to result in the formation of oil-insoluble products not suitable for the present invention. It also appears that aromatic constituents oxidize more readily than do the non-aromatic components. Thus, failure to remove the most aromatic materials from the feed before oxidation results in formation of considerable oil-insoluble materials. Usually a suitable petroleum fraction, upon distillation under reduced pressure, e. g., molecular distillation, will produce a first 10 percent by weight fraction which has a viscosity of more than 50 SUS at 210° F., preferably more than 80 SUS at 210° F.

The lubricating oils, such as highly refined petroleum bright stocks which are employed in the oxidation reaction to prepare the stabilizing additive, can be additionally treated so as to yield a desired solid product of improved color properties as more fully disclosed and claimed in the U. S. application by W. B. Whitney, Serial No. 264,840, filed January 3, 1952, now U. S. Patent No. 2,786,803 issued March 26, 1957. The additive material which is produced without this type of treatment is very dark red in color. An outstanding improvement resulting from this additional treatment is that the stabilized additive is much lighter in color than a product obtained without this treatment and does not produce as dark a color in a liquid hydrocarbon fuel composition containing the same.

Broadly speaking, this additional treatment comprises treating the charge stock prior to oxidation by contacting it with silica gel or a similar solid selective adsorbent for the removal of the more aromatic hydrocarbon types. Accordingly a lubricating oil stock such as a petroleum bright stock which has substantially no asphalt, a low aromatic content and, preferably, low wax content, is additionally treated with silica gel at about room temperature, usually in the range 40° F. to 70° F., and a sufficient pressure differential is maintained across the bed or mass of silica gel so as to cause a satisfactory flow therethrough of the lubricating oil fraction being treated. The charge stock which is thus treated may be any hydrocarbon fraction suitable for the production of the additive of this invention, usually a hydrocarbon fraction having a viscosity in the range 70 to 700 SUS at 210° F., preferably a lubricating oil fraction in the range 115 to 300 SUS at 210° F. A highly refined lubricating oil in these ranges will generally have an average molecular weight in the range 550 to 1100. It is preferred that the hydro-

carbon fraction contain no portion having a molecular weight below 450.

It has been found that materials which are useful as stabilizing additives in liquid hydrocarbon fuels and which are useful as ashless detergents in lubricating oils are produced by oxidation of such an above-described selected hydrocarbon fraction. During the oxidation reaction for the production of the additive material, the selected hydrocarbon fraction is modified, resulting in a product of increased dispersant activity which differs from the starting material in respect to the four following physical characteristics

- (1) An increase in the carbon to hydrogen weight ratio
- (2) An increase in molecular weight
- (3) An increase in the oxygen content
- (4) A decreased solubility in propane under propane fractionating conditions

All these changes are brought about by contacting an above-described selected hydrocarbon fraction under suitable conditions of temperature and pressure with an oxidizing agent such as free oxygen, sulfur trioxide, nitrogen dioxide, nitrogen trioxide, nitrogen pentoxide, acidified chromium oxides and chromates, permanganates, peroxides such as hydrogen peroxide, sodium peroxide and ozone. Any oxygen containing material capable of releasing free oxygen under the oxidizing conditions may be used. Suitable other specific oxidizing agents include air, relatively pure commercial grade oxygen, oxygen enriched air, and a mixture of oxygen with an inert gas, such as carbon dioxide and nitrogen. Even oxygen admixed with natural gas or methane is satisfactory. Air having less than the usual amount of oxygen may also be used. Air is economically a preferred oxidizing agent.

Generally the oxidation reaction is carried out at a temperature in the range of from -40° F. to 800° F. When using an active oxidizing agent such as sulfur trioxide, temperatures in the range of -40° F. to 400° F., preferably 70° F. to 200° F. are used. With less active oxidizing agents, such as air, higher temperatures are used, such as 100° F. to 800° F., preferably 390° F. to 575° F. Higher oxidation temperatures result in a faster oxidation reaction. When the oxidizing agent is in the gaseous phase, another variable which affects the rate of the oxidation reaction is the partial pressure of the oxidizing agent. Accordingly, as the pressure at which the oxidation reaction is carried out is increased, other conditions remaining the same, the oxidation reaction proceeds at a faster rate. Therefore, depending upon the rate of oxidation desired, the oxidation reaction is carried out at sub-atmospheric, atmospheric or super-atmospheric pressure. Usually it is preferred to carry out the oxidation reaction at a pressure between about 10 and 100 lbs. per square inch absolute depending upon the composition or oxygen content of the oxidizing gas. Lower or higher absolute pressures may be satisfactorily used if desired. Lower oxidation pressures are useful in that they facilitate release and removal of the more volatile, and other undesirable materials, e. g., H<sub>2</sub>O from the reaction mixture.

The rate of oxidation is also dependent upon and influenced by the distribution of the oxidizing gas within the reaction mixture and the rate of introduction of the oxidizing gas thereto. The oxidizing agent is preferably introduced and present in the reaction mixture in a finely dispersed state in order to achieve better contact with the materials undergoing oxidation and better mixing therewith. An increase in the rate of introduction of the oxidizing gas of course increases the rate of oxidation, other conditions remaining unchanged. The conditions of temperature, pressure, oxygen content of the oxidizing gas, rate of introduction of oxidizing gas, etc., are correlated, adjusted and controlled so as to carry out the oxidation reaction at a sufficiently rapid rate so as to

minimize reaction time while readily and easily controlling the reaction.

Conditions which have been found to be satisfactory for producing the stabilizing additive from a selected hydrocarbon fraction when using a moderate oxidizing agent, such as air, are set forth in Table 3.

TABLE 3

|                         | Reaction Condition                                                                                  | Broad Range | Preferred |
|-------------------------|-----------------------------------------------------------------------------------------------------|-------------|-----------|
| 10                      |                                                                                                     |             |           |
| Temperature, ° F.       | 100-800                                                                                             | 375-575     |           |
| Time of Oxidation, hrs. | 3-75                                                                                                | 5-60        |           |
| Pressure, p. s. i. a.   | 10-200                                                                                              | 15-100      |           |
| 15                      | Rate of introduction of oxidizing agent in s. c. f. (standard cubic feet) per pound of oil per hour | 0.01-3.0    | 0.04-0.4  |

Exemplary of the influence of various variables upon the oxidation reaction, it is pointed out that at a temperature of 482° F. and at an air introduction rate of about 0.32 s. c. f. per pound of oil per hour and at about atmospheric pressure, the oxidation reaction requires about 20 hours before the desired degree of completion is reached (as measured by increase in viscosity). When the air rate was increased to 1.44 s. c. f. per pound of oil per hour, only 16 hours were required to convert the oil to an oxidized product of similar viscosity. Increasing the reaction temperature to 572° F. decreased the time required for oxidation appreciably. Reducing the reaction temperature to below 390° F. increased the reaction time under these conditions.

More active oxidizing agents, such as sulfur trioxide may also be used in the oxidation step as pointed out above. When liquid sulfur trioxide is utilized as the oxidizing agent, the reaction is most readily carried out when both the oil and sulfur trioxide are separately diluted with a modifying solvent. Solvents which may be utilized in this operation under suitable temperature conditions include liquid sulfur dioxide, hexane, tetrachloroethylene, ethylene dichloride, pyridine, nitrobenzene and dioxane.

Liquid sulfur trioxide is an extremely reactive compound and, if added directly to the oil, will cause excessive charring and violent splattering. It is necessary to moderate this excessive reactivity by dilution with a solvent such as those disclosed above. A molar ratio of solvent to sulfur trioxide of at least about 1:1 appears to be necessary and it is preferred to use a ratio of 2:1 or greater. Dilution of the oil is also very desirable for the reduction of viscosity and to facilitate mixing, but such a dilution is not required. Dilution of the oil may be obtained with some non-reactive solvent other than that utilized for the dilution of the sulfur trioxide. Use of the same diluent, however, simplifies the recovery problem. Gaseous SO<sub>3</sub> may be introduced into the oil directly or mixed with a carrier gas such as air, nitrogen or other inert gas. In the case of gaseous SO<sub>3</sub> an elevated temperature, e. g., 200 to 300° C., may be used.

The extent of oxidation is determined by the ratio of oil to sulfur trioxide. The weight ratio may be varied from 1:1 to 30:1 but is preferably maintained within the range of between 3:1 to 18:1. Ratios from 3:1 to 8:1 are the most desirable. Very low ratios result in the use of excessive amounts of sulfur trioxide without obtaining a corresponding increase in useful product. Very high ratios fail to obtain sufficient oxidation to be economical.

The initial reaction of the sulfur trioxide with oil is almost instantaneous at room temperature or above, but reaction continues for extended periods of time, e. g., up to as much as 144 hours or more. At higher temperatures, the time of the slower secondary reactions is shortened to less than 24 hours. The evolution of sulfur dioxide and other gases causes much foaming and the rate of reaction must be controlled sufficiently to

permit the capacity of the apparatus to handle the foaming reaction mixture. The time required for reaction may be shortened to as little as three minutes, in which case, secondary reactions do not take place to any great extent. The quality of the product is not materially affected by the length of reaction time or by the absence or occurrence of the secondary reactions.

The temperatures which may generally be utilized in the oxidation reaction, wherein sulfur trioxide is used as the oxidizing agent, range from  $-40^{\circ}$  F. to  $400^{\circ}$  F., 10 preferably from  $70^{\circ}$  F. to  $200^{\circ}$  F. A very short period of time, usually less than three hours, is required for the initial reaction.

After the reaction, the product is treated for the removal of acid and other impurities. Acid is conveniently removed from the product by water washing. The product is concentrated in the manner discussed later in connection with the product obtained in a process utilizing a less active oxidizing agent.

The additive produced by sulfur trioxide oxidation is somewhat improved in color by reduction. This is preferably accomplished by treatment in alcohol with lithium hydride or with zinc and hydrochloric acid. Catalytic hydrogenation or chemical reduction may also be used.

The extent to which the oxidation reaction is carried out is dependent upon the selected oil fraction being oxidized and the yield of additive material desired. I have found that if the oil being oxidized contains a relatively low concentration of lower molecular weight hydrocarbons the oil may be oxidized to a considerable extent, up to as high as 75 percent by weight of the oil charged, without any deleterious effects upon the reaction itself or the additive material. Also I have observed that when the aromatic content of the charge stock is low, such as below about 5 percent by weight of carbon atoms in aromatic rings and especially below about 2 percent by weight, the charge stock can be oxidized to a greater extent without any undesirable effects or adversely affecting the yield such as may happen when there is an appreciable amount, above about 5 percent by weight of aromatic carbon atoms present therein. In general, the oxidation reaction is carried out until the oxidized oil has increased in viscosity, when expressed in Saybolt Universal seconds (SUS) at  $210^{\circ}$  F., from 0.5 to 50 fold, preferably from 3 to 10 fold, over that of the originally charged unoxidized oil. When the oxidation reaction is carried out to a 3 to 10 fold increase in viscosity the yield of active stabilizing additive recovered from the oxidized oil amounts to about 15 to 50 percent by weight of the original unoxidized oil. Continued oxidation, especially above about 60 percent, tends to produce a certain amount of oil-insoluble oxidized materials which, although they do not adversely affect the effectiveness of the oil-soluble additive, do adversely affect the yield of the desired product. Also since it is often necessary to remove these oil-insoluble oxidized materials, it is desirable therefore not to continue the oxidation reaction beyond that point at which the oil-insoluble materials are produced.

The stabilizing additive of this invention produced during the oxidation reaction dissolves in the lubricating oil from which it is prepared since it is oil soluble. The oxidized reaction mixture itself is useful as the hydrocarbon fuel additive since it possesses the stabilizing properties when added to or compounded with that fuel. It is often desirable to prepare a concentrate of the active solid additive material which comprises substantially only the solid additive material. This active solid additive material can be recovered directly from the oxidized reaction mixture by solvent extraction with a solvent which is selective for the relatively unoxidized, essentially hydrocarbon material therein and which solvent is at the same time essentially a non-solvent for the active additive material in the reaction mixture. Suitable solvents for the recovery of the solid active additive

material from the oxidized reaction mixture include propane, isopropyl alcohol, a solvent mixture of propane with modifying amounts (up to about 50 percent by weight) of other low boiling hydrocarbons such as methane, ethane, and butane. Other selective solvents such as methyl ethyl ketone, methyl isobutyl ketone, tertiary butyl alcohol, isobutyl alcohol, ethyl acetate, dioxane, morpholine, dimethyl formamide, phenol and isopropyl alcohol are also useful. In general those polar compounds containing only carbon, hydrogen, and oxygen atoms, such as aliphatic alcohols, aliphatic ketones, and esters having from 3 to 8 carbon atoms per molecule are useful as treating materials in the practice of this invention. Mixtures of these various materials may be used.

One step-wise process for concentrating the additive material comprises extracting the partially oxidized oil with methyl isobutyl ketone, methyl ethyl ketone or mixtures of the two at appropriate temperatures so as to dissolve only the oil and lower molecular weight oxidation material. The proper temperature will depend upon the ratio of solvents and the percentage of product to be dissolved. The undissolved material is thereafter mechanically separated from the dissolved material.

When these materials are used in obtaining the active additive material from the oxidized reaction mixture, the active solid additive is recovered as a propane insoluble, oil soluble, solid phase (raffinate), the ineffective, substantially hydrocarbon material of the reaction mixture being dissolved in the treating material as an extract. The propane soluble phase from which the active additive material is separated has a viscosity index much higher than that of the unoxidized oil. This propane soluble phase may be used to blend with an oil for the purpose of improving the viscosity index of that oil.

In the recovery of the active additive material, it is preferred in the practice of this invention to employ propane as a selective solvent, the solid active additive being recovered as a separate propane insoluble phase under propane fractionating conditions of temperature, pressure and ratio of solvent to material being treated (usually 5:1 to 25:1 by vol.). The solvent extraction operation for the recovery of the active additive material is usually carried on at a temperature in the range  $50^{\circ}$  F. to  $250^{\circ}$  F. especially in the range  $100^{\circ}$  F. to  $160^{\circ}$  F. and a pressure of between 200 p. s. i. g. to 500 p. s. i. g. Countercurrent solvent extraction techniques are usefully employed as well as multiple, solvent extraction steps of separately contacting and recovering the undissolved active additive.

In many instances, the activity of the additive material is considerably increased by additionally treating this recovered solid additive material with an aliphatic alcohol, in the  $C_3$  to  $C_8$  range, such as isopropyl alcohol, and recovering a purified and more active additive therefrom as a solid, alcohol insoluble phase. The alcohol treatment has a two-fold purpose. Traces of peroxides, aldehydes, and the like which may be oxidation promoters are removed thereby. In addition thereto, it appears that a beneficial chemical change takes place during stripping of residual alcohol solvent from the additive material.

The above-described sequence of recovery and purification steps does not in some instances greatly influence the quality and effectiveness of the solid, final additive product. It is preferred to employ a propane fractionation step prior to the organic polar compound treating step to avoid emulsions which are difficult to break and which present operational difficulties when the alcohol or ketone treating step precedes the propane solvent extraction step.

Normally liquid hydrocarbon fuel to which this stabilizing additive is added may be any of the fuels ranging through the gasoline boiling range to and through the fuel oils and diesel fuel range and even as high as

720° F. Although fairly large quantities of this additive will tend to discolor the fuel to which it is added, it should be noted that I utilize only a maximum of 0.1 weight percent of this additive to obtain the stabilization desired. Such a quantity of additive material does not materially affect the color of the fuel, i. e., gasoline. It is particularly beneficial, however, to utilize the silica gel treatment discussed hereinabove, so as to produce as light a product as possible and thus the color of the additive material before its incorporation into the normally liquid hydrocarbon fuel.

The stabilizing additive disclosed hereinabove is more fully disclosed and discussed in the U. S. application of W. B. Whitney, Serial No. 304,659, filed August 15, 1952, now abandoned. In that application, the product of oxidation has been disclosed as being useful as an ashless detergent in lubricating oil.

The following examples are illustrative of the subject invention and of the advantages to be obtained in the practice thereof. These examples are not intended to be unduly limitative of this invention.

#### Example I

The stabilized additive used in the following examples was prepared as follows: 403 pounds of finished 250 lubricating oil blending stock were charged to a 50 gallon still. Air was passed through the oil in the still at a rate of 7 standard cubic feet per minute. The pressure was adjusted to 25 p. s. i. g. and the temperature to 482° F. and held there throughout the run. The run was continued until the viscosity of the oil had increased to about 350 SUS at 210° F. At the conclusion of the run, which required 10.6 hours, a liquid overhead product of 12.9 pounds had been collected and consisted of two phases, i. e., an aqueous phase of 8.4 pounds and an oil phase of 4.5 pounds.

The oxidized oil was withdrawn from the still and was charged to a propane fraction column which was operated under the conditions and with the results set forth in Table I.

TABLE I.—PRIMARY PROPANE FRACTIONATION

|                                            |     |
|--------------------------------------------|-----|
| Top column temp., ° F.....                 | 150 |
| Oil charge temp., ° F.....                 | 132 |
| Propane charge temp., ° F.....             | 115 |
| Bottom column temp., ° F.....              | 110 |
| Column pressure, p. s. i. g.....           | 450 |
| Oil charge rate, G. P. H. @ 60° F.....     | 2.2 |
| Propane to oil ratio, vol. (estimate)..... | 5.8 |
| On stream time, hrs.....                   | 21  |

| Products      | lbs.  | wt. percent of charge | 2.0 Vis., SUS | Rd @ 70 C. | Color |
|---------------|-------|-----------------------|---------------|------------|-------|
| overhead..... | 283.1 | 80.6                  | 184.7         | 1.4806     | 8+    |
| bottoms.....  | 68.3  | 19.4                  |               |            |       |
|               | 351.4 | 100.0                 |               |            |       |

All of the overhead product from the above described propane fractionation was charged to a 50 gallon batch still. The oxidation air rate was adjusted to 5.8 s. c. f. per minute. The pressure raised to 25 p. s. i. and the temperature raised to 482° F. and held there throughout the run. The run was continued until the viscosity of the oil had increased to about 600 SUS at 210° F. At the conclusion of the run, 21.1 pounds of liquid overhead product had been collected which consisted of 12.2 pounds of aqueous phase and 8.9 pounds of oil phase.

The oxidized oil from the secondary oxidation was charged to a propane fractionation column. Table II presents data on this fractionation step.

TABLE II.—SECONDARY PROPANE FRACTIONATION

|                            |     |
|----------------------------|-----|
| Top column temp., ° F..... | 150 |
| Oil charge temp., ° F..... | 132 |

|                                            |      |
|--------------------------------------------|------|
| Propane charge temp., ° F.....             | 115  |
| Bottom column temp., ° F.....              | 110  |
| Column pressure, p. s. i. g.....           | 450  |
| Oil charge rate, G. P. H. @ 60° F.....     | 2.2  |
| Propane to oil ratio, vol. (estimate)..... | 6.0  |
| On stream time, hrs.....                   | 12.7 |

| Products      | lbs.  | wt. percent of charge | 2.0 Vis., SUS | Rd @ 70 C. | Color |
|---------------|-------|-----------------------|---------------|------------|-------|
| overhead..... | 139.5 | 66.2                  | 155           | 1.4765     | 8+    |
| bottoms.....  | 71.4  | 33.8                  |               |            |       |
|               | 210.9 | 100.0                 |               |            |       |

The bottoms product of this fractionation constituted the stabilizing additive and the material used in the following examples.

#### Example II

Filtering tests were made on a fuel oil with and without the stabilizing additive of a fuel with a 50:50 blend of light cycle oil and straight run stove oil. The filter test was conducted in a jet fuel filtering apparatus.

The test procedure utilized was as follows: A fuel reservoir containing a sample of the fuel was connected to the apparatus and a slight air pressure was applied to the fuel so as to force it into the filtering system. Bubbles were worked out of the flow lines and the flow regulator was adjusted so that a flow of 6.0 milliliters per minute per square centimeter of square filter area was obtained. A total of 50–100 milliliters of fuel was allowed to pass through the system at room temperature to equilibrate it. The relay was deactivated and the pinch clamp was closed. The temperature of the filter bath was adjusted to 70° F. and after the fuel in the filter bath had been raised to the desired temperature, flow was resumed by reactivating the relay and opening the pinch clamp. The filtrate was received in a graduated cylinder and readings were taken for each 10 milliliters filtered so that a curve relating pressure and volume could be plotted. The filter is considered clogged for a jet fuel when the pressure drop across the filter reaches 260 milliliters' mercury pressure. This value varies when fuels other than a jet fuel are used in the filtering apparatus. Table III gives the data obtained by filtering of oil aged at 150° F. for 14 days in dark, glass storage with and without the stabilizing agent.

TABLE III.—VOLUME FILTERED VS. PRESSURE DROP

| Volume Filtered ml. of fuel oil | Pressure Drop (mm. Hg)   |                                        |                                        |
|---------------------------------|--------------------------|----------------------------------------|----------------------------------------|
|                                 | Aged Fuel (No Detergent) | Aged Fuel 0.0005 wt. Percent Detergent | Aged Fuel +0.001 wt. Percent Detergent |
| 10.....                         | 18                       | 4                                      | 0                                      |
| 20.....                         | 40                       | 4                                      | 2                                      |
| 30.....                         | 60                       | 4                                      |                                        |
| 40.....                         | 80                       | 8                                      | 6                                      |
| 50.....                         | 100                      | 8                                      |                                        |
| 60.....                         | 120                      | 8                                      | 10                                     |
| 80.....                         | 166                      | 10                                     | 16                                     |
| 100.....                        | 208                      | 14                                     | 24                                     |
| 120.....                        | 240                      | 18                                     | 32                                     |
| 140.....                        | 280                      | 24                                     | 40                                     |
| 160.....                        | 314                      | 28                                     | 50                                     |
| 180.....                        | 360                      | 34                                     | 60                                     |
| 200.....                        | 392                      | 40                                     | 72                                     |
| 250.....                        |                          | 54                                     | 100                                    |
| 300.....                        |                          | 72                                     | 130                                    |
| 350.....                        |                          | 86                                     | 162                                    |
| 400.....                        |                          | 108                                    | 192                                    |
| 450.....                        |                          | 128                                    | 220                                    |
| 500.....                        |                          | 160                                    | 236                                    |

*Example III.—Procedure for determining fuel oil insoluble residue by filtration*

**A. Apparatus:**

- (1) Gooch-type Pyrex crucible with fritted glass disk having a porosity of 14 microns
- (2) Filter flask, 250 ml., equipped with funnels and rubber crucible holders

**B. Reagents:**

- (1) ASTM naphtha
- (2) Acetone
- (3) Nitric acid, concentrated
- (4) Sulfuric acid, concentrated

A Gooch crucible was thoroughly cleaned by immersing it in a hot acid bath (maintained at 240° F. to 280° F.) consisting of approximately 3 parts concentrated nitric acid and one part concentrated hydrochloric acid. After the crucible was allowed to remain in the hot bath for 2 hours, it was cooled and rinsed thoroughly with tap water, distilled water, and finally with acetone. This was followed with a one-hour drying period in an oven at 150° C. Crucible was then transferred to a cooling vessel and allowed to cool for at least one hour before weighing. A sample of distillate fuel in the amount of 100 ml. was filtered by suction through the weighed Gooch crucible. Crucible was then transferred to another filter flask. The vessel which contained the sample of fuel oil was then washed with three portions of ASTM naphtha and the washings were added to the crucible after each rinse. Following this step, the outside and the bottom of the Gooch crucible were carefully washed with ASTM naphtha to remove all traces of oil. Crucible was then dried for one hour at 150° C., transferred to a cooling vessel and allowed to cool for 2 hours before reweighing. Residue was the increase in weight calculated as milligrams per 100 ml. of sample.

The data are given in Table IV.

TABLE IV.—INSOLUBLE GUM  
[Aged at 150° F. for 14 days in dark glass bottles.]

|                                             | Insoluble Gum<br>Before<br>Aging | (mg./100<br>ml.) |    |
|---------------------------------------------|----------------------------------|------------------|----|
| (1) Blend with no additive.....             | 0.9                              | 4.7              | 45 |
| (2) (1) + 0.0005 wt. percent detergent..... | 0.4                              | 2.1              |    |
| (3) (1) + 0.001 wt. percent detergent.....  | 1.8                              | 1.9              |    |

From the data set forth in the above examples, it is clear that gum formation is readily inhibited in the

50

normally liquid hydrocarbon fuel. Various modifications of this invention will be apparent to those skilled in the art, but such modifications are believed to be clearly within the spirit and the scope of this invention.

5 I claim:

1. A stabilized fuel consisting essentially of normally liquid hydrocarbon and between 0.0001 and 0.01 weight percent of a gum-formation-inhibiting oxygenated component obtained by oxidation of an aliphatic hydrocarbon fraction in which the ratio of carbon atoms to olefinic bonds is at least 16:1, having a refractive index  $n_D^{20}$  in the range of 1.440 to 1.520, an average molecular weight in the range of 550 to 10,000 and substantially all components thereof having a minimum molecular weight of 450, a viscosity in the range of 50 to 1400 SUS at 210° F., a viscosity index (when determinable) in the range of 50 to 125 and an average carbon atom content per molecule in the range of 40 to 720.

2. The fuel of claim 1 in which said component has an acid number below 50, a saponification number in the range of 0-100, and an oxygen content in the range of 1 to 15 weight percent.

3. The stabilized fuel of claim 1 wherein said normally liquid hydrocarbon has a boiling range below 720° F.

25 4. The fuel defined in claim 1 further characterized in that said hydrocarbon fraction is obtained from a topped, distilled, and vacuum reduced crude and is substantially free of asphalt.

5. The fuel defined in claim 1 further characterized in that said hydrocarbon fraction is obtained from a topped, distilled, and vacuum reduced crude substantially free of asphalt by propane fractionation and solvent extraction to remove aromatics.

30 6. A gasoline having dissolved therein a small but 35 gum inhibiting amount of an oil soluble, propane insoluble, isopropyl alcohol insoluble, solid, oxygenated hydrocarbon.

References Cited in the file of this patent

UNITED STATES PATENTS

|    |           |                |       |               |
|----|-----------|----------------|-------|---------------|
| 40 | 2,070,567 | Adams          | ----- | Feb. 16, 1937 |
|    | 2,081,176 | Hewlett et al. | ----- | May 25, 1937  |
|    | 2,337,336 | McCluer et al. | ----- | Dec. 21, 1943 |
|    | 2,472,152 | Farkas et al.  | ----- | June 7, 1949  |
|    | 2,575,003 | Caron et al.   | ----- | Nov. 13, 1951 |
|    | 2,667,408 | Kleinholz      | ----- | Jan. 26, 1954 |
|    | 2,758,069 | Whitney        | ----- | Aug. 7, 1956  |
|    | 2,786,803 | Whitney        | ----- | Mar. 26, 1957 |

UNITED STATES PATENT OFFICE  
CERTIFICATE OF CORRECTION

Patent No. 2,875,029

February 24, 1959

Leo A. McReynolds

It is hereby certified that error appears in the printed specification of the above numbered patent requiring correction and that the said Letters Patent should read as corrected below.

Column 4, line 64, for "40° F. to 70° F." read -- 40° F. to 170° F. --.

Signed and sealed this 29th day of December 1959.

(SEAL)  
Attest:

KARL H. AXLINE  
Attesting Officer

ROBERT C. WATSON  
Commissioner of Patents